

Dec. 13, 1932.

J. ASTON ET AL

1,890,637

METHOD OF MAKING WROUGHT IRON

Filed July 19, 1928

Fig. 1.



Fig. 2.



Fig. 3.



INVENTOR

James Aston  
A. H. Keale  
By James Stith Penick & Ford  
Their Atty's

## UNITED STATES PATENT OFFICE

JAMES ASTON AND ADDISON H. BEALE, OF PITTSBURGH, PENNSYLVANIA, ASSIGNEES,  
BY MESNE ASSIGNMENTS, TO A. M. BYERS COMPANY, OF PITTSBURGH, PENNSYLVANIA, A CORPORATION OF PENNSYLVANIA

## METHOD OF MAKING WROUGHT IRON

Application filed July 19, 1928. Serial No. 294,048.

Our invention relates to the Aston process of making wrought iron, such, for example, as set forth in several United States patents of James Aston, such as No. 1,370,507, granted March 8, 1920, for method of making wrought iron pipe; No. 1,412,823, granted April 18, 1922, for method of making wrought iron; and No. 1,469,373, granted October 2, 1923, for manufacture of wrought iron.

An object of the invention is to provide for the formation by the Aston process of a wrought iron sponge or ball having a shape adapting it for particular purposes and insuring substantially complete granulation of the metal, even toward the end of the pour. For these purposes a ball having at least one horizontal dimension greater than its vertical dimension is formed.

20 A further object of the invention is to improve the efficiency and economy of the Aston process by re-using of the molten slag employed in the shotting or granulating operations. As previously carried out, in operating the Aston process of making wrought iron, a large mold was partially filled with molten slag of the desired puddling characteristics, the liquid product of the steel-making process was poured into it to cause granulation of the steel due to the temperature difference between the steel and the slag bath, and the puddled iron ball was collected in the bottom of the mold. The excess slag was then poured off and the puddle ball dumped out. In such method of operation the excess slag solidified and its heat was wasted.

We have found that we can increase the economy and efficiency of the process by re-using the molten slag a plurality of times, thus avoiding much of the expense of remelting. In carrying out our improved method, we prefer to employ a large cup or pot of ferrous material which is of such dimensions and so designed that it can be and is lined with firebrick or other refractory material. The lined receptacle which we prefer to employ is about 3 feet by 4 feet in interior cross-sectional dimensions, and about 4½ to 5 feet deep. A larger receptacle may be used if a larger puddle ball is desired.

In the drawing:

Figure 1 is a plan view of one form of receptacle for carrying out my invention; and

Figures 2 and 3 are vertical cross sections on the lines II—II and III—III, respectively, of Figure 1.

In this drawing, 2 represents an iron or steel receptacle preferably formed with trunnion lugs 3—3. This receptacle is preferably cast with an upper inwardly projecting lip 60 or flange 4, if it is to be lined with firebrick, such as shown at 5.

In the form shown, the sides diverge upwardly, two of the sides diverging more sharply than the other two sides. The bottom dimensions of the lined vessel are about four feet along the longer axis by about three feet along the shorter axis.

Sufficient slag is poured into this receptacle to fill it to about one-half or two-thirds full. The receptacle should contain sufficient slag so that its temperature will be conserved to the degree desired in the process, and so that the excess slag can be re-used while in the liquid or molten state. The preferred depth of slag is about 3 feet. It is important to provide a sufficient depth of slag bath, in order to give the granules a proper distance of travel so that they have sufficient time to release their contained oxides and gases into the slag bath before contacting with the wrought iron ball or mass at the bottom and welding and building up the wrought iron sponge. This desirable time element is obtained by the proper depth of bath. After the pouring in of the steel is completed, the gases which cause more or less foaming or boiling, pass off and the level of the bath usually lowers while the last granules are descending and welding with the spongy mass at the bottom.

The vessel is of such size in at least one horizontal dimension that a ball of desirable weight may be formed having at least one horizontal dimension greater than its vertical dimension. Such a ball is particularly well adapted for formation in a hydraulic press into a bloom of suitable size and shape for rolling into slabs or billets, and by reason of the shape of the ball a sufficient depth of

slag is maintained over it, even toward the end of the pour, to insure substantially complete granulation of the metal in the overlying slag.

During the pouring operation, the temperature of the slag is somewhat increased by reason of the relatively high temperature of the steel entering it. For proper operation, the slag must be kept sufficiently cool to properly solidify and granulate the steel, several hundred degrees' difference being requisite for this purpose. We have found that by lining the vessel with refractory material the slag remaining above the ball is maintained sufficiently hot so that it can be poured out into another cup or receptacle. After the shotting operation, the surplus slag is poured into the next cup or receptacle and the puddle ball is then dumped out and goes to the press.

In the second cup or receptacle the same operations may be carried out. After the puddle ball is formed therein the slag may be again poured out into a third cup or receptacle and the slag thus re-used a number of times.

The advantages of our invention result from the formation of a ball having at least one horizontal dimension greater than its vertical dimension, which is particularly suited for pressing into a bloom of desired size and shape and insures substantially complete granulation of the metal, even toward the end of the pour, from the re-use of the slag while in molten condition, thus conserving its heat, and further from the use of refractory or heat-insulating material in connection with the pouring receptacle, thus conserving the heat of the slag.

Many changes may be made in the form of the receptacle, the steps in the process, etc., without departing from our invention.

We claim:

1. In the manufacture of wrought iron, the steps consisting of feeding molten ferrous material through a molten slag bath in a receptacle, and forming in the lower portion of the receptacle a ball having at least one horizontal dimension greater than its vertical dimension.

2. In the manufacture of wrought iron, the steps consisting of feeding granulated ferrous material through a molten slag bath in a receptacle, forming in its lower portion an elongated ball having one horizontal dimension greater than its vertical dimension, pouring off the surplus slag directly into another receptacle, again feeding granulated ferrous material therethrough to form another horizontally elongated ball, and removing the ball from the first receptacle and compressing it.

3. In the manufacture of wrought iron, the steps which comprise feeding a stream of molten ferrous material into a bath of molten

slag in a receptacle and producing a horizontally elongated ball of metal and slag in the bottom of the bath while maintaining a sufficient depth of slag over the metal to assure the granulation of the metal at the end of the pour, thereafter tilting the receptacle and pouring off the surplus slag, allowing the slag to drain from the ball, collecting the slag in another receptacle and feeding ferrous material through the bath of slag in the second receptacle while the slag is still molten.

4. In the manufacture of wrought iron, the steps consisting of feeding granulated ferrous material through a molten slag bath, conserving the heat of the bath by reducing heat losses therefrom, feeding the surplus slag while molten into another receptacle, and repeating the operation therein.

5. In the manufacture of wrought iron, the steps consisting of feeding granulated ferrous material through a molten slag bath, retarding the loss of heat through the walls of the receptacle, tilting the receptacle to feed the surplus slag while molten into another receptacle, retarding the heat losses through the second receptacle, removing the ball from the first receptacle and then compressing it, and pouring molten ferrous material into the slag in the second receptacle.

6. In the manufacture of wrought iron the steps consisting of feeding granulated ferrous material through a molten slag bath in a receptacle, retarding the heat losses through the walls of the receptacle, removing surplus slag while molten and feeding it into a second receptacle, retarding the heat losses through the walls of the second receptacle, removing the ball from the first receptacle and then compressing it, and feeding granulated ferrous material through the slag bath in the second receptacle while the same is still molten.

7. In the manufacture of wrought iron, the steps consisting of feeding hot granules of ferrous material through a molten slag bath in a receptacle having one transverse dimension greater than another, retarding heat losses through the walls of the receptacle, removing the surplus slag and the capsule from the receptacle, and feeding the slag into another receptacle, retarding heat losses through the walls of the second receptacle and compressing the capsule removed from the first receptacle.

In testimony whereof we have hereunto set our hands.

JAMES ASTON.  
ADDISON H. BEALE.